

Jan. 15, 1935.

W. S. NUTTER ET AL

1,987,632

MOHAIR WARP YARN AND METHOD OF PRODUCING SAME

Filed June 8, 1933

Fig1.

Fig2.

Fig3.



Inventors.  
William S. Nutter  
Clifford Holdsworth  
by *Heard Smith & Tennant.*  
Atlys.

## UNITED STATES PATENT OFFICE

1,987,632

MOHAIR WARP YARN AND METHOD OF  
PRODUCING SAME

William S. Nutter, Sanford, and Clifford Holdsworth, Springvale, Maine, assignors to Goodall Worsted Company, Sanford, Maine, a corporation of Maine

Application June 8, 1933, Serial No. 674,959

9 Claims. (Cl. 117—52)

This invention relates to a new construction of yarn and to a new method of producing yarn whereby a mohair or similar fibre yarn equal or superior to yarns now in use for corresponding purposes may be produced much more rapidly and economically than such yarns have heretofore been produced. While the yarn of this invention may be employed for a wide variety of purposes, it has marked advantages when employed as a warp yarn and particularly as the pile warp in the weaving of warp pile fabrics, such, for example, as mohair plush or velvet.

While various systems are employed for spinning yarn from cotton fibres and from mohair and other animal fibres, there are well-known and markedly distinctive differences between the systems employed particularly in the cost and speed of operation as between the cotton spinning systems and the systems for spinning mohair and animal fibres due primarily to the characteristic differences in the fibres themselves.

Cotton fibres are relatively short and hence it is impossible in the spinning operation to give the relatively long draft and tight twist characterizing the spinning of mohair and similar fibres as by the Bradford or worsted systems. In cotton spinning, the required tightness and twist is obtained both by the twist imparted in the spinning of the single yarn and by the doubling and twisting of yarns of single count into ply yarns. But owing to the nature of the fibre, the spinning operations are performed far more rapidly and economically than in the case of the spinning operations in the spinning of mohair and other animal fibres.

In the spinning of mohair yarn by the systems heretofore employed, the finer the count to which the yarn is spun, the less is the proportion of the fleece which can be utilized and a point is reached at which the proportion of the fleece wasted becomes so great that the cost of the yarn becomes excessive.

One of the objects of the present invention is to utilize in the spinning of mohair yarn in part the principles heretofore employed in the spinning of cotton yarn, thus greatly increasing the rapidity with which the yarn may be produced and greatly reducing the cost of manufacture.

In this invention the yarn is partially produced by a spinning operation involving the principles of cotton spinning and partially by a spinning operation involving the principles of the mohair or worsted spinning systems heretofore employed and with the entire elimination of the separate twisting operation heretofore employed with the

result that the yarn produced is of the nature of a single yarn but of the count of a corresponding ply yarn, of ample strength for the required purposes, and of distinctive and superior characteristics as hereinafter set forth.

The drawing illustrates conventionally the yarn and certain steps in the method of its production.

In the drawing:

Fig. 1 is a perspective view of the single yarn strand.

Fig. 2 is a perspective view of the strand of mohair roving.

Fig. 3 is a perspective view of the finished yarn. It will be understood that it is impossible in a drawing to show the exact proportions, dimensions of the yarn and its component parts and the exact arrangement, proportions and dimensions of the fibres in the yarn. The drawing therefore only serves to illustrate in a general way the construction and is entirely of a conventional nature.

In carrying out the invention, the minimum amount of cotton fibre is introduced that is necessary to enable the yarn to be produced partly by the cotton spinning methods and hence far more rapidly and economically than heretofore. Moreover, the cotton fibre content is so located in the finished yarn as not materially to detract from its appearance, feel and other characteristics as compared with the mohair yarn spun by the usual processes.

In carrying out the invention, a single yarn strand represented by Fig. 1 is first spun on the regular cotton system from a roving composed of a mixture of cotton fibres and mohair fibres with the mohair content in the maximum proportion that is practical to enable the strand to be thus spun. It is well known that it is impractical to spin a mixed cotton and mohair yarn with the methods employed in cotton spinning and at the same time have the mixture contain more than approximately 50% mohair fibre and consequently in the preferred practice of the invention in spinning this strand the roving is composed of substantially equal parts of cotton and mohair fibres. In the broader aspect of the invention the non-cotton content may be composed partially of wool or other animal fibre but when the mohair is thus mixed with such other fibre, the primary consideration is one of fibre cost.

In the production of this single yarn strand, the mohair fibres should first be cut to substantially the same length as the staple of the cotton fibres employed. This strand is spun not only rapidly and economically, due to the use of the

methods employed in cotton spinning, but this strand utilizes a maximum amount of the mohair fleece because of the relatively short fibre length necessary to mix with the cotton fibre.

5 In carrying out the invention, the single yarn strand thus spun is next doubled with a strand of mohair roving represented by Fig. 2 and then these two strands are spun together by the methods heretofore employed in spinning mohair yarn 10 such, for example, as the well-known Bradford or worsted spinning system, but with this noteworthy distinction, that in this spinning operation the single yarn strand is not subjected to any draft, while the mohair roving is given a 15 draft in the usual manner. This is accomplished by guiding the single yarn strand out of the drafting rolls of the spinning frame while allowing the mohair roving strand to pass through the drafting rolls in the usual manner.

20 The results are that the twist given by the spinning operation is imparted partially to the roving strand and that this strand is wrapped around and caused to envelop the single yarn strand in helical form. The mohair roving strand when it 25 enters this spinning operation has, of course, only a very slight twist or only that necessary to hold the fibres together and consequently a very substantially less twist than in the single yarn strand. At the conclusion of the spinning operation, 30 the mohair strand therefore envelops the single yarn strand in a helix of less turns per unit length than there are in the twist of the other strand.

35 The finished yarn represented by Fig. 3 has the appearance, feel and characteristics of a single mohair yarn with a minor proportion of cotton fibre lying at the center.

40 In the production of the yarn, the weight per unit length of the two strands employed is preferably the same.

The roving strand in certain forms of the invention may be a mixture of mohair and other suitable animal fibre. But in this case a further and important subsidiary feature of the invention 45 resides in that this roving strand is preferably composed of a mixture in which there is a major proportion of mohair fibre and a minor proportion of fine wool fibre. It will be recognized that in the finished yarn of this invention there is very 50 much less total twist in the yarn and its component strands as compared with a two-ply mohair yarn spun by the methods heretofore employed and that particularly there is much less twist in the enveloping strand imparted thereto 55 by the final spinning operation employed herein than in either component single yarn of a corresponding two-ply mohair yarn spun by the previous methods. Consequently by utilizing in this 60 enveloping strand a suitable proportion of fine wool fibre, this wool fibre as it is twisted with the mohair fibre acts to enwrap and lay into the strand the ends of the mohair fibres which otherwise are apt to project and render the yarn more or less "wild". The proportion of fine wool fibre 65 thus employed to secure this result is readily determined depending upon the particular character of the two fibres employed and the extent to which smoothness in the finished yarn is required.

70 It will be recognized that with this invention there has been no separate twisting operation employed and that the yarn has been produced entirely by spinning operations. Thus the entire 75 expense of twisting machinery with the cost and

time required for the twisting operation is eliminated.

Furthermore, it will be recognized that the enveloping roving strand may be spun down to a fine count with a minimum wastage of the mohair content because of the way in which it is spun in this invention. If, for example, this strand were spun as a single yarn on the worsted system or the methods heretofore employed, it could only be spun to about half the count that it can be spun as a strand of the yarn of this invention and still utilize without wastage the same proportion of the mohair fleece. Putting it concretely, if the enveloping roving strand be spun as a single yarn on the worsted system to, say, a 16-count, only that portion of the mohair fleece could be utilized without wastage which would be utilized by spinning the same strand to a 32-count as a part of the yarn of this invention.

While, as noted, the yarn of this invention may be used for a wide variety of purposes, it has distinctive advantages when employed as the pile warp in the manufacture of cut warp pile fabric. In the two-ply mohair yarn heretofore 25 employed for this purpose, each ply is, of course, separately twisted in the spinning operation and the two plies are twisted together in the twisting operation. When this yarn is woven in to form the pile of the fabric and the loops are cut, this 30 twist is not entirely released and is, in fact, only released part way down from the cut portion of the pile. Consequently there is an essential impairment of the desired smooth velvety appearance. With the yarn embodying the present invention employed in the manufacture of similar goods, when the pile loops are cut, the twist, which, as heretofore pointed out, is very much less than in the previous case, is practically entirely released down to the bottom of 40 the pile so that a remarkably smooth velvety appearance is imparted to the pile fabric. In fact it is found in practice possible to weave the fabric with a lower pile and consequently with the utilization of a lesser amount of yarn in the 45 case of yarn made in accordance with the present invention as compared with the yarns made by previous methods and to obtain superior results.

Again it will be noted that in the yarn of the 50 present invention the cotton content is introduced only to enable the utilization of the cotton spinning methods with the consequent great reduction in time and cost of manufacture. This cotton content lies at the center of the yarn and does not materially affect the appearance, feel and characteristics of the yarn as compared with a yarn containing no cotton content. This is particularly noticeable in the case of the pile fabrics referred to because when the pile loops are cut, the ends of the cut pile are practically entirely of mohair fibre. Due to the greater resiliency or spring of the mohair fibre, these fibres stand far above the cotton fibres which retract practically to the base of the pile. Hence in such a cut pile fabric woven with the yarn of this invention, the appearance, feel and characteristics of the fabric are practically the same as those of an all-mohair cut pile fabric and in addition 70 a lesser amount of the yarn is required and the appearance of the fabric is markedly enhanced by reason of the practically complete release of the twist in the pile.

Having thus described the invention, what is

- claimed as new, and desired to be secured by Letters Patent, is:
1. The method of forming yarn which consists in forming a mixture of cotton and animal fibres in which the animal fibres are wholly or partially mohair and in which the maximum length of all the fibres is the maximum length of the cotton fibres, forming a roving from the said mixture, spinning a single yarn strand in the way in which cotton yarn is spun from the said roving, forming a roving of animal fibres in which the animal fibres are wholly or partially of mohair, and in which the average length of the fibres is essentially greater than the average length of the fibres in the first roving, doubling with the spun single yarn strand the second strand of roving, and spinning together the two strands without drafting the spun single yarn strand while drafting the second roving strand to cause the latter to envelop the former. 10
  2. A yarn composed of a twisted core strand of a mixture of cotton and animal fibres in which the animal fibres are wholly or partially mohair, and in which the maximum length of all the fibres is the maximum length of the cotton fibres, and a twisted enveloping strand of animal fibres in which the animal fibres are wholly or partially of mohair and in which the average length of the fibres is essentially greater than the average length of the fibres in the core strand, the enveloping strand having a markedly less twist than the core strand and enveloping the core strand in a helix of less turns per unit length than in the twist of the core strand. 15
  3. A yarn composed of a twisted core strand of a mixture of substantially equal amounts of cotton and animal fibres in which the animal fibres are wholly or partially mohair, and in which the maximum length of all the fibres is the maximum length of the cotton fibres, and a twisted enveloping strand of animal fibres in which the animal fibres are wholly or partially of mohair and in which the average length of the fibres is essentially greater than the average length of the fibres in the core strand, the enveloping strand having a markedly less twist than the core strand and enveloping the core strand in a helix of less turns per unit length than in the twist of the core strand. 20
  4. A yarn composed of a twisted core strand of a mixture of cotton and animal fibres in which the animal fibres are wholly or partially mohair, and in which the maximum length of all the fibres is the maximum length of the cotton fibres, and a twisted enveloping strand of a mixture of mohair fibres and fine wool fibres, in which the wool fibres constitute the minor component and in which the average length of the mohair fibres is essentially greater than the average length of the fibres in the core strand, the enveloping strand having a markedly less twist than the core strand and with the wool fibres enwrapping and holding in the enveloping strand the bulk of the ends of the mohair fibres of the said strand. 25
  5. A yarn composed of a twisted core strand of a mixture of substantially equal amounts of cotton and animal fibres in which the animal fibres are wholly or partially mohair, and in which the maximum length of all the fibres is the maximum length of the cotton fibres, and a twisted enveloping strand of a mixture of mohair fibres and fine wool fibres, in which the wool fibres constitute the minor component and in which the average length of the mohair fibres is essentially greater than the average length of the fibres in the core strand, the enveloping strand having a markedly less twist than the core strand and with the wool fibres enwrapping and holding in the enveloping strand the bulk of the ends of the mohair fibres of the said strand. 30
  6. A yarn composed of a spun strand of a mixture of substantially equal amounts of cotton and animal fibres in which the animal fibres are wholly or partially mohair and in which the maximum length of all the fibres in the core strand is the maximum length of the cotton fibres, and an enveloping strand of roving of animal fibres in which the animal fibres are wholly or partially mohair and in which the average length of the fibres in the enveloping strand is essentially greater than the average length of the fibres in the core strand, the core strand lying in an unextended condition in the yarn and the enveloping strand lying in a slightly twisted condition and in a helix about the core strand. 35
  7. A yarn composed of a twisted core strand of a mixture of substantially 50% of cotton fibres and 50% mohair or mohair and wool fibres and in which the maximum length of all the fibres is the maximum length of the cotton fibres, and a twisted enveloping strand of mohair fibres having an average length essentially greater than the average length of the fibres in the core strand, the enveloping strand having a markedly less twist than the core strand and enveloping the core strand in a helix of less turns per unit length than in the twist of the core strand. 40
  8. A yarn composed of a twisted core strand of a mixture of substantially 50% of cotton fibres and 50% mohair or mohair and wool fibres and in which the maximum length of all the fibres is the maximum length of the cotton fibres, and a twisted enveloping strand of a mixture of mohair fibres and fine wool fibres, in which the wool fibres constitute the minor component and in which the average length of the mohair fibres is essentially greater than the average length of the fibres in the core strand, the enveloping strand having a markedly less twist than the core strand and enveloping the core strand in a helix of less turns per unit length than in the twist of the core strand and with the wool fibres enwrapping and holding in the enveloping strand the bulk of the ends of the mohair fibres of the said strand. 45
  9. A yarn composed of a twisted core strand of a mixture of substantially equal amounts of cotton fibres and mohair fibres in which the cotton and mohair fibres are of substantially the same length, and a twisted enveloping strand of a mixture of mohair fibres and fine wool fibres, in which the wool fibres constitute the minor component and in which the average length of the mohair fibres is essentially greater than the average length of the fibres in the core strand, the enveloping strand having a markedly less twist than the core strand and enveloping the core strand in a helix of less turns per unit length than in the twist of the core strand and with the wool fibres enwrapping and holding in the enveloping strand the bulk of the ends of the mohair fibres of the said strand. 50
  - 70
  - 75